

## 1

3,464,840

**CELLULOSE-SULFUR COMPOSITION WHICH  
RESISTS CHAIN SHORTENING**

Donald M. MacDonald, Hawesbury, Ontario, Canada, assignor to Canadian International Paper Company, Montreal, Quebec, Canada, a corporation of Canada  
No Drawing. Filed Jan. 4, 1965, Ser. No. 423,317  
Int. Cl. C08b 27/64

U.S. CL. 106—162

## 3 Claims

**ABSTRACT OF THE DISCLOSURE**

A stable composition comprising a cellulosic material, alkali, and sulfur in an amount of from about 0.1% to 2.0% by weight of the cellulosic material.

This invention relates to the production of cellulose having greater average chain lengths. More particularly, it relates to a method of inhibiting the breaking down of cellulose chains during aging or other reactions.

The processes required for the manufacture of articles of commerce from regenerated cellulose or from cellulose ethers may be divided into several distinct steps. Usually, although the present invention is not intended to be restricted to this process, the following steps are followed:

(a) Purified cellulose, either wood pulp or cotton linters, in sheet form, is placed in strong (about 18%) sodium hydroxide solution. Subsequently, the sheet may be broken up by vigorous agitation (slurry process) or allowed to remain undisturbed in the caustic solution (sheet steeping process). After a predetermined time, varying from seconds to hours, the excess caustic is drained off and the cellulose mass pressed to remove further caustic. The pressed mass, now known as alkali cellulose, is shredded and broken up into small fragments or almost to individual fibers. This shredding step can also be carried out at the end of step (b) infra;

(b) The alkali cellulose is allowed to "age" for a predetermined time and at a predetermined temperature;

(c) The aged alkali cellulose is treated with carbon disulfide (xanthated) and dissolved at the end of the reaction time in dilute caustic soda (sodium hydroxide solution). The solution is known as viscose. Alternatively, the alkali cellulose can be treated with ethylene oxide to produce hydroxyethyl cellulose, with chloroacetic acid to produce carboxymethyl cellulose, or in other manners known to those skilled in the art.

Cellulose, when treated with strong alkali, undergoes a complex reaction with atmospheric oxygen and with alkali. The main feature of this reaction is a shortening of the molecular chain length by breakage at random positions. This reaction continues in the above process until such time as the cellulose derivative is dissolved in water or in more dilute caustic soda, or is freed from strong caustic by any means. The extent of the chain shortening is governed by the time and temperature used in step (b). Even if step (b) is eliminated, chain shortening occurs at all times in steps (a) and (c) when the cellulose is in contact with strong caustic.

In many instances, it is desirable that the chain shortening, or aging reaction, be minimized. Such instances occur, for example, in the production of cellulose sausage casings, in the production of high wet modulus rayons of the Toramomen type, and in the production of cellulose ethers when prepared from cellulose following a strong caustic treatment and for use as viscosity increasers for aqueous solutions. In the first two instances, very desirable strength properties are obtainable if the average cellulose chain length is kept as great as possible and, in the last instance, the longer the average chain length the less cellulose ether is required for a given solution viscosity increase.

## 2

(The term "aging reaction" as used herein refers not just to step (b) but to all chain shortening processes due to the actions of alkali and atmospheric oxygen in any procedure in which cellulose is treated with solutions of caustic stronger than about 7%. For economic reasons, the preferred base is sodium hydroxide, rather than hydroxides of lithium, potassium, or caesium, but these can also be used.)

It is known that alkali metal sulfites (U.S. Patent No. 1,857,948, to R. Dosne, dated May 10, 1932), certain heavy metal salts (Entwistle, Cole and Wooding, Text. Res. J., 19,609–624 (1949)); Sihlola and Bostrom, Paper and Timber, 34, 23–27 (1952), sodium borohydride (Swedish Patent 162,095 to I. Jullander dated Feb. 11, 1958), polyhydric phenols (German patent application No. ST 3147 filed Mar. 12, 1951 by Dr. Hermann Staudinger), sodium trithiocarbonate (U.S. Patent 2,473,954 dated June 21, 1949 to G. M. A. Kayser), and gluconic or mucic acids (Canadian Patent 563,087 dated Sept. 9, 1958 to W. R. Saxton) can inhibit chain shortening in the aging reaction.

None of these materials has enjoyed wide use as all suffer from objections. Sodium sulfite is soluble in steeping lye and must be added after pressing unless very large quantities are used. Sodium trithiocarbonate also suffers from this objection and is not chemically stable. Sodium borohydride is also unstable and, on decomposition, generates hydrogen causing an explosion hazard. Polyhydric phenols turn brown in caustic and cause undesirable colors in the final product. The heavy metal salts may also give objectionable color and can cause difficulties in filtration of solutions of the products. Gluconic and mucic acids are primarily intended to combat the accelerating effect of accidentally introduced catalytic heavy metal ions, and these acids are soluble in steeping lye.

It is a principal object of this invention to provide a really effective inhibitor of chain shortening during the aging reaction which is not subject to the noted objections.

It has now been found that sulfur can be added to cotton linters or wood pulp before either is subjected to sheet or floc formation and that the sulfur is retained by the pulp. The sulfur is not soluble in a steeping lye and there is accordingly no contamination problem. Moreover, it does not cause difficulties in filtration of solutions of cellulose xanthate and has no detectable harmful effect on the color or strength of the final product. The sulfur can also be added to caustic prior to bringing the caustic into contact with cellulose or to alkali cellulose prior to bringing the alkali caustic into contact with carbon disulfide in xanthation. But, for best results, it should be added as early as possible, preferably no later than at the start of the shredding operation, so as to assure even dispersal of the sulfur throughout the mass.

Quantities of sulfur ranging from about 0.1 to 2.0% based on the weight of cellulose effectively inhibit aging. The preferred amount is 1% by weight.

The following examples are not intended to restrict the invention in any way, but are offered merely as illustrations of the effectiveness of the present invention. The figures under "D.P." (degree of polymerization) indicate the average number of monomer units of cellulose per chain at the specified time. The viscose viscosity is well known to be proportional to the average chain length, so that these figures give an idea of the overall effect of the sulfur.

**Example I**

A sulfite wood pulp of dissolving grade in sheet form (specifically, "Tenacell" grade pulp manufactured at the Kipawa Mill of Canadian International Paper Company) was treated with a solution of sulfur in carbon disulfide. The added weight of sulfur was 1% based on cellulose.

This pulp was dried until no trace of carbon disulfide remained and was subsequently converted to alkali cellulose by sheet steeping in 18% sodium hydroxide solution. After draining and pressing, the alkali cellulose contained 32% cellulose. A sheet of this alkali cellulose was torn into small pieces and thoroughly dispersed in an about 5% aqueous acetic acid solution (this step causes cellulose to be reformed from the alkali cellulose). The D.P. of the cellulose after thorough washing was determined from its viscosity in cuprammonium hydroxide solution.

The bulk of the alkali cellulose was shredded for 60 minutes and a second sample of cellulose was regenerated for D.P. determination. A third sample was regenerated after aging for 24 hours, after which time the remaining alkali cellulose was treated with carbon disulfide (about 33% CS<sub>2</sub>) and converted to cellulose xanthate. The cellulose xanthate was dissolved in an aqueous alkali solution to yield a viscose containing 5% cellulose and 6% sodium hydroxide. The ball fall viscosity in seconds of this viscose was determined after ripening for 48 hours.

For comparison purposes, a second experiment starting with sulfur-free pulp was carried out in which 1% sulfur was added at the alkali cellulose shedding stage. A third experiment in which no sulfur was added was also carried out. Care was taken to insure that temperatures and times were identical at each stage of the three experiments. Results were as follows:

TABLE I.—EFFECT OF 1% SULFUR ON THE AGING REACTION

| Amount added<br>(Percent of cellulose weight) | When added              | DP after— |           |          | Viscose viscosity (sec.) |
|-----------------------------------------------|-------------------------|-----------|-----------|----------|--------------------------|
|                                               |                         | Pressing  | Shredding | 24 hours |                          |
| 0                                             |                         | 770       | 763       | 468      | 16.2                     |
| 1                                             | Cellulose before alkali | 811       | 766       | 545      | 44.6                     |
| 1                                             | Shredding stage         | 778       | 760       | 490      | 31.1                     |

Reduction of chain shortening with sulfur is indicated, as is the advantage of early addition of the sulfur.

TABLE III.—AGING INHIBITION CAUSED BY VARIOUS AMOUNTS OF SULFUR

| Amount of sulfur added<br>(percent of cellulose weight) | DP after— |           |          | Viscose viscosity (sec.) |
|---------------------------------------------------------|-----------|-----------|----------|--------------------------|
|                                                         | Pressing  | Shredding | 24 hours |                          |
| 2                                                       | 781       | 764       | 568      | 50.0                     |
| 1                                                       | 769       | 763       | 560      | 50.8                     |
| 0.5                                                     | 783       | 767       | 556      | 36.2                     |
| 0.25                                                    | 785       | 767       | 554      | 31.8                     |
| 0                                                       | 783       | 767       | 503      | 21.2                     |

10

## Example IV

0.10% by weight of sulfur is also an active inhibitor, as was illustrated following addition in CS<sub>2</sub> solution to a prehydrolyzed hardwood sulfate pulp of dissolving grade. The CS<sub>2</sub> was completely removed by drying before contact with caustic. In this preliminary experiment, only the viscose viscosity was determined. The viscose from treated pulp had a viscosity of 122 seconds, while an untreated control had a viscosity of 116 seconds.

20

## Example V

Aging was inhibited when a prehydrolyzed sulfate pulp (specifically "Tyrecell" grade pulp manufactured at the 25 Natchez Mill of International Paper Company) and cotton linters pulp were used as cellulosic raw materials. All conditions in the following runs, including method of

TABLE V.—INHIBITION USING LINTERS AND PREHYDROLYZED SULFATE PULP

| Pulp                  | Percent sulfur | D.P. after— |           |          | Viscose viscosity (sec.) |
|-----------------------|----------------|-------------|-----------|----------|--------------------------|
|                       |                | Pressing    | Shredding | 24 hours |                          |
| Prehydrolyzed sulfate | 1              | 730         | 721       | 571      | 50.6                     |
| Do                    | 0              | 728         | 722       | 549      | 31.6                     |
| Linters               | 1              | 682         | 620       | 520      | 28.6                     |
| Do                    | 0              | 639         | 625       | 469      | 15.2                     |

## Example II

The sulfur used in Example I was an unpurified grade such as is commonly used in the preparation of wood pulp. Two purer grades have also been tried at the 1% level while in CS<sub>2</sub> solution in an experiment using the techniques given in Example I.

## Example VI

The purified sulfite pulp of Example I in sheet form was soaked in water overnight. Each soaked sheet was 55 then slurried in water by 5 seconds stirring with a high speed mixer of the Osterizer type. Sulfur (1%) was added in dry form to the pulp slurry which was stirred a further

TABLE II.—RESULTS USING PURIFIED SULFUR

| Amount added<br>(percent of cellulose weight) | Type and grade of sulfur   | DP after— |           |          | Viscose viscosity (sec.) |
|-----------------------------------------------|----------------------------|-----------|-----------|----------|--------------------------|
|                                               |                            | Pressing  | Shredding | 24 hours |                          |
| 0                                             |                            | 787       | 769       | 502      | 19.6                     |
| 1                                             | U.S.P. Grade, precipitated | 791       | 767       | 567      | 52.1                     |
| 1                                             | N.F. Grade, sublimed       | 788       | 768       | 568      | 53.0                     |

Table II shows that the degree of inhibition effected by these purer grades of sulfur is of the same order as found in Example I.

## Example III

Using the pulp and procedures of Example I, the effect of the addition of different amounts of U.S.P. grade sulfur to pulp was studied.

15 seconds at the high speed. The slurry, which contained 70 0.3% cellulose, was diluted with ten volumes of water using hand or mild mechanical stirring for 30 seconds. The diluted pulp slurry was poured onto a screen, and excess water allowed to drain. Drained water was used in the preparation of the next sheet. Make up water only 75 was added. The wet sheet on the screen was pressed and

passed through a set of wringers of the type used in home washing machines to remove all loosely retained water. The new pulp sheets were dried, conditioned, and processed essentially in the same manner as in Example I. The control sheets were prepared as above except that no sulfur was added and fresh water was used. Water remaining after preparation of both the control and sulfur handsheets was tested for sulfur by shaking with sulfur-free carbon disulfide. A drop of pure mercury added to the carbon disulfide did not turn black or change color in any way in either case. This proves that there was little or no contamination of the water with sulfur (Feigl: Spot Tests in Inorganic Analysis, 5th edition, 374, Elsevier Publishing Company).

Caustic drained and expressed from the above sheets 15 during alkali cellulose pressing was retained and reused in steeping a second batch of the original sheets of the same pulp.

TABLE VI.—RESULTS OBTAINED USING SULFUR-CONTAINING HAND-SHEETS AND AFTER REUSING EXPRESSED CAUSTIC (COMBINED DRAININGS AND PRESSINGS)

| Batch No.                      | Type and amount of sulfur<br>(percent of cellulose weight) | DP after— |           |             | Viscose<br>viscosity<br>(sec.) |
|--------------------------------|------------------------------------------------------------|-----------|-----------|-------------|--------------------------------|
|                                |                                                            | Pressing  | Shredding | 24<br>hours |                                |
| 1                              | 1% U.S.P. sulfur, handsheets                               | 782       | 769       | 535         | 36.8                           |
| 2                              | 1% N.F. sulfur                                             | 770       | 770       | 523         | 36.2                           |
| 3                              | None, handsheets                                           | 773       | 750       | 468         | 16.9                           |
| Caustic Recovered from 1, none |                                                            | 785       | 778       | 511         | 28.2                           |
| Caustic Recovered from 2, none |                                                            | 785       | 765       | 515         | 26.8                           |
| Caustic Recovered from 3, none |                                                            | 814       | 765       | 512         | 25.7                           |

The results from the first three lines of the table clearly show the inhibiting effect of the sulfur. The results obtained when expressed caustic was used with fresh, un-dispersed pulp (last three lines of Table VI) show that little or no sulfur leaves the alkali cellulose during caustic removal. The generally higher level of results from recovered caustic when compared to the control handsheets results indicates that catalytic iron originally present (5 p.p.m.) has been removed from the sodium hydroxide solution by the pulp in the previous steeping.

#### Example VII

It is shown by Example IV that sulfur inhibits alkali cellulose aging but does not influence the catalytic effect of heavy metal impurities in caustic or pulp. This was illustrated further when a purer caustic is used in steeping. This caustic contained 0.7 p.p.m. iron rather than the 5 p.p.m. present in the caustic used in all other examples.

TABLE VII.—RESULTS WHEN PURE CAUSTIC WAS USED

| Amount of sulfur used (percent of cellulose weight) | DP after— |           |             | Viscose<br>viscosity<br>(sec.) |
|-----------------------------------------------------|-----------|-----------|-------------|--------------------------------|
|                                                     | Pressing  | Shredding | 24<br>hours |                                |
| 1                                                   | 778       | 772       | 598         | 77.0                           |
| 0                                                   | 785       | 775       | 538         | 34.2                           |

Note, by comparison with Table I, that the control 24 hour D.P. and viscose viscosity are higher in Table VII, due to use of caustic containing less catalytic iron. However, the inhibitor effectiveness judging by the viscosity and 24 hour D.P. increase achieved with the presence of sulfur is almost unchanged. Had the sulfur acted by prevention of iron catalysis, very little inhibition should have been found in the presence of only 0.7 p.p.m. of iron.

#### Example VIII

The sulfite dissolving grade wood pulp was treated with 1% sulfur, steeped in caustic, and shredded as in Example I. A sulfur-free control was also processed using the same conditions. No samples were taken for D.P. determination.

The sulfur-containing pulp was aged for three days at 28° C. and the sulfur-free pulp was aged for three days at 23° C. The aged alkali celluloses were xanthated and

5 dissolved in caustic to give viscose containing 7% cellulose and 6% NaOH. The viscose had ball fall viscosities of 38 seconds. If both alkali cellulose samples had been aged at 25° C., experience shows that 106 and 67 hours would have been required to reach a viscosity of 38 seconds. Using the formula

Percent change in aging =

$$\frac{(\text{Aging time sulfur} - \text{aging time control}) 100}{\text{Aging time control}}$$

10 this corresponds to 58% longer aging when sulfur is used at the 1% level, based on cellulose.

Viscose color and transparency, cellulose yield, and sheet steeping properties (such as floating, cracking, and processing absorption—all well known to those learned in the art of cellulose sheet steeping) were all identical between the samples. The two viscose filtered with equal ease and were spun after ripening into a bath containing

130 g. of H<sub>2</sub>SO<sub>4</sub>, 16 g. of ZnSO<sub>4</sub>, and 280 g. of Na<sub>2</sub>SO<sub>4</sub> per liter. The rayons had excellent color and strength after washing and drying. No differences were found.

#### Example IX

Percent increase in viscose viscosity has been determined for many of the inhibitors mentioned in the literature. The sulfite pulp used in most of the above examples was used here also and percent increases were calculated by the formula:

Percent viscose viscosity increase =

$$\frac{100 (\text{viscose viscosity, inhibitor} - \text{viscose viscosity, control})}{\text{Viscose viscosity, control}}$$

40 All processing parameters were as given in Example I and viscosities of control batches varied by not more than ±4.0 seconds.

TABLE IX.—PERCENT VISCOSITY INCREASE CAUSED BY SULFUR AND A VARIETY OF OTHER MATERIALS MENTIONED AS INHIBITORS IN THE LITERATURE

| Inhibitor               | Amount used | Where added                             | Percent viscose viscosity increase |
|-------------------------|-------------|-----------------------------------------|------------------------------------|
| Sodium borohydride      | 1%          | Reacted with pulp <sup>1</sup>          | 17.3                               |
| Do                      | 0.05%       | do <sup>1</sup>                         | 0                                  |
| Copper ethyl xanthate   | 250 p.p.m.  | Pulp                                    | 22.2                               |
| Pyrogallol <sup>3</sup> | 1%          | Steeping caustic                        | 60.0                               |
| Do <sup>5</sup>         | 4.1%        | Shredder                                | 26.2                               |
| Sodium sulfite          | 1%          | Steeping caustic                        | 16.2                               |
| Do                      | 1%          | Shredder                                | 61.8                               |
| Potassium sulfite       | 1%          | Steeping caustic                        | 19.4                               |
| Do                      | 1%          | Shredder                                | 58.3                               |
| Lithium sulfite         | 1%          | Steeping caustic                        | 20.3                               |
| Do                      | 1%          | Shredder                                | 40.6                               |
| Sulfur                  | 1%          | Xanthation CS <sub>2</sub> <sup>4</sup> | 37.5                               |
| Do                      | 1%          | Shredder                                | 92.0                               |
| Do                      | 1%          | Pulp                                    | 175                                |

55 1 No inhibition was found when 1.0 and 0.05% sodium borohydride was added to the caustic at steeping time.

2 Large amounts are not practical because of reagent insolubility.

3 A polyhydric phenol.

4 25% solution in 18% NaOH.

5 As shown in expired U.S. Pat. No. 1,689,958 to Moro.

#### Example X

A sample of sulfite dissolving pulp, specifically Filmcell H, manufactured at the Hawkesbury mill of the Canadian International Paper Company, was treated with a 75 solution of sulfur in carbon disulfide. The added weight

of sulfur was 1% based on cellulose. This pulp was dried until no trace of carbon disulfide remained and was then converted to alkali cellulose by slurry steeping in 18% sodium hydroxide. After draining and pressing the alkali cellulose, containing 34% cellulose, was shredded and aged for three days at 25° C. After this time, the alkali cellulose was reacted with ethylene oxide gas (11% based on cellulose) simply by rotating the glass storage vessel at room temperature while connected to another vessel containing the required amount of liquid ethylene oxide. The ethylene oxide vaporized and was completely absorbed into, and reacted with, the alkali cellulose after two hours. The hydroxyethyl cellulose was dissolved in dilute caustic soda to give a solution containing 8% hydroxyethyl cellulose and 7% NaOH. The solution was frozen overnight, thawed, and allowed to come to 20° C. before the viscosity was determined.

A control batch of the same pulp was converted to alkali cellulose, then to hydroxyethyl cellulose, and dissolved simultaneously and using identical procedures to those used for the sulfur-containing pulp. The hydroxyethyl cellulose solution prepared using the pulp containing 1% sulfur had a viscosity of 52.6 secs. while the con-

tro1 batch containing no sulfur had a viscosity of 12.2 secs.

What is claimed is:

1. A stable composition comprising a cellulosic material, alkali, and sulfur in an amount of from about 0.1% to 2.0% by weight of the cellulosic material.
2. A composition as in claim 1 wherein the cellulosic material is selected from the group consisting of cotton linters, wood pulp and alkali cellulose.
3. A composition as in claim 2 wherein the sulfur is present in an amount of about 1% by weight.

#### References Cited

##### UNITED STATES PATENTS

|           |        |        |       |         |
|-----------|--------|--------|-------|---------|
| 1,857,948 | 5/1932 | Dosne  | ----- | 260—233 |
| 2,473,954 | 6/1949 | Kayser | ----- | 260—233 |

DONALD E. CZAJA, Primary Examiner

R. W. MULCAHY, Assistant Examiner

U.S. Cl. X.R.

260—231, 233